

# UNITED STATES PATENT OFFICE.

EMIL BRONNERT, OF NIEDERMORSCHWEILER, NEAR MÜLHAUSEN, AND MAX FREMERY, OF OBERBRUCH, GERMANY.

## PROCESS FOR PRODUCING CELLULOSE PRODUCTS.

1,030,251.

Specification of Letters Patent.

Patented June 18, 1912.

No Drawing.

Application filed December 24, 1907. Serial No. 407,972.

*To all whom it may concern:*

Be it known that we, EMIL BRONNERT, a subject of the Emperor of Germany, residing at Niedermorschweiler, near Mülhausen, in Alsace, Germany, and MAX FREMERY, a subject of the King of Prussia, residing in Oberbruch, Germany, have invented a certain new and Improved Process for Producing Cellulose Products, of which the following is a specification.

Cellulose threads have previously been produced by spinning a cuprammonia cellulose solution into a caustic soda bath to precipitate the cellulose and subsequently eliminating the copper from the threads after a preliminary washing of the latter to remove the soda and ammonia. The threads were then dried under tension in the usual manner. For certain purposes the copper cellulose threads could be dried directly, but care has always been necessary to avoid the decomposition of the cellulose with resulting injury to the strength of the threads. This old process produces a thread containing cellulose and copper in simple molecular proportion. We have now discovered that a thread containing much less copper, (to one molecule of cellulose, but two-thirds or even only one-half a molecule of copper) may be obtained by the use of a precipitating bath of novel composition and action, namely one which not only precipitates the cellulose by the use of the customary caustic soda, but also contains a substance which combines with and separates out at least portion of the copper in the precipitated cellulose filament.

Among suitable substances for the last mentioned purpose may be mentioned glucose, saccharose, lactose and their equivalents. A suitable quantity of one of these substances, preferably saccharose, is added to a precipitating bath containing the usual quantity of caustic soda. The bath may for example contain 32 grams of caustic soda, and 8 grams of saccharose to each 100 cubic centimeters of water. The jet of cuprammonia cellulose solution which is "spun" into this bath is at once precipitated or coagulated, by the action of the soda. A part of the copper of the so formed filament being substituted by sodium and saccharose, the ammonia is eliminated, part of the copper is at once dissolved and precipitated under the reducing action of the sugar in the pres-

ence of alkali (soda) preferably at the temperature (approximately 45° C. to 70° C.) at which the process is carried on. The precipitating bath is rapidly colored brick-red by the suspended cuprous oxid so that any threads that happen to tear off are readily discovered. These filaments coming from the precipitating bath comprise cupric-cellulose or a cupric-sodic-cellulose compound. After having been washed in the usual manner to remove the caustic soda, during which much of the dissolved copper is also washed out, the threads which are of a malachite green of fine transparent brilliancy, may be directly and quickly dried under tension at a temperature of even 100° C. The remaining copper is withdrawn at any time from the dry threads by washing with diluted (e. g. 2%) sulfuric acid.

It will be seen that the action of the saccharose is not that of a precipitant, for which purpose it has been previously proposed, although it is practically impossible to produce a filament in a saccharose or similar solution however concentrated it may be. The saccharose plays a very different part, namely it combines with portion of the copper to form a substance which is dissolved out of the thread and reduced at once by the hot alkaline bath. It has also been proposed to use a dilute sulfuric acid precipitating bath to which is added sugar or glucose or glycerin to arrest the injurious action of the acid upon the filament. But this in no way suggests the present bath in which no acid is employed and in which consequently there is no noxious acid action to prevent. Moreover the threads produced are of entirely distinct chemical composition—the hydrocellulose of the acid bath being neither as strong as nor in any way as desirable as the cupric cellulose thread obtained by the present process. Furthermore, the proposal to use an alkaline glycerin precipitating bath, which has been made, has not been of any value, since it was not understood that glycerin *per se* is not a coagulant—and is useless unless the bath contain soda in sufficient strength to effect the precipitation of the cellulose in the manner described.

Filaments similar to those produced by the present process, having only a low copper content, have never previously been produced with a soda precipitating bath.

We claim as our invention:

1. In the process of manufacturing cellulose products from cuprammonium solutions of cellulose, the introduction of the latter in suitable form into a precipitating bath containing caustic soda as the precipitant and a sacchariferous substance which combines with at least portion of the copper present in the precipitated cellulose thread to form a compound, which is carried away from the thread and then immediately reduced in the presence of soda in the alkaline bath, substantially as described.
2. In the process of manufacturing cellulose products from cuprammonium solutions of cellulose, the introduction of the latter in suitable form into a precipitating bath having a temperature of from 45° C. to 75° C. and containing caustic soda as the precipitant and a sacchariferous substance which combines with at least portion of the copper present in the precipitated cellulose thread to form a compound carried away from the thread and then immediately reduced in the presence of soda in the bath, substantially as described.
3. In the process of manufacturing cellulose products from cuprammonium solutions of cellulose, the introduction of the latter in suitable form into a precipitating bath containing caustic soda as the precipitant and a sacchariferous substance which combines with at least portion of the copper present in the precipitated cellulose thread to form a compound carried away

from the thread and then immediately reduced in the presence of soda in the bath, and thereafter washing the thread to remove the soda and then drying under tension.

4. In the process of manufacturing cellulose products from cuprammonium solutions of cellulose, the introduction of the latter in suitable form into a precipitating bath containing caustic soda as the precipitant and a sacchariferous substance which combines with at least portion of the copper present in the precipitated cellulose thread to form a compound dissolved out from the thread and then immediately reduced in the presence of soda in the bath, and thereafter washing the thread to remove the soda and then eliminating the remaining copper and sugar from the thread by washing in dilute (say 2%) sulfuric acid and drying under tension.

5. A filament of the character described, precipitated from a cuprammonium solution of cellulose by introduction into a bath of caustic soda containing sugar and having its copper content subsequently removed, substantially as described.

In testimony whereof we have signed our names to this specification, in the presence of two subscribing witnesses.

EMIL BRONNERT.

MAX FREMERY. [L. S.]

Witnesses:

OTTO KÖNIG,

WILHELM FRIEDERICH.